

# UNITED STATES PATENT OFFICE.

AUGUST H. PRINZ AND HERMANN HABER, OF VIENNA, EMERICH TOMISCHKA, OF HIRSCHWANG, AND JOSEF FREIHERR VON BRENNER, OF VIENNA, AUSTRIA-HUNGARY.

## METHOD OF TREATING JUTE-BAST, &c.

SPECIFICATION forming part of Letters Patent No. 621,135, dated March 14, 1899.

Application filed December 31, 1897. Serial No. 665,221. (No specimens.)

*To all whom it may concern:*

Be it known that we, AUGUST H. PRINZ and HERMANN HABER, of Vienna, EMERICH TOMISCHKA, of Hirschwang, and JOSEF FREIHERR VON BRENNER, of Vienna, Austria-Hungary, have invented certain new and useful Improvements in the Method of Treating Jute-Bast and the Like for Use in Textile Industries, of which the following is a specification.

10 Our invention has for its object the extraction of cellulose from plant fibers without the aid of heat in order to better adapt such fibers for use in textile industries.

By way of example we shall in the following 15 description apply our process to the extraction of fibers from jute-bast, although we may in a similar manner extract fibers from chinagrass, rheia, and other vegetable matter.

In the mechanical treatment of the crude 20 jute-bast the sticks of jute are loosened by mechanical means with a machine of known construction. The loosened jute-bast is freed by hand or by machinery from the tips and root ends in order to obtain the jute-bast in 25 as uniform a state as possible. In the chemical treatment the jute-bast mechanically treated in the manner above described is first subjected to a macerating process in an alkaline solution and without the aid of heat.

30 We have discovered in the course of our experiments that caustic-soda lyes are most suitable and economical for use in a macerating process. To macerate without the aid of heat, we use, by way of example, caustic-soda lyes having a specific gravity of 1.035, and we have noticed that the concentration of the macerating-lyes varies according to the quality of the jute-bast under treatment.

This macerating process is carried on in the 40 following manner: The jute-bast, cut into lengths of about from one to 1.5 meters and freed from root ends and tips, is laid lengthwise in a sheet-iron receptacle having a double perforated bottom and an outlet-cock. Five cubic meters of crude jute-bast may, by way of example, be placed in such a receptacle. After having thus laid the jute-bast in the reservoir the caustic-soda lyes, of a specific 45 gravity of 1.035, are added thereto—say, for

instance, seven hundred liters (in volume) of 50 such lyes to one hundred kilos of crude jute-bast.

To operate with economy—that is to say, to carry on the treatment with the smallest possible quantity of caustic-soda lyes—we proceed by successive stages in the following manner, for instance: In the first stage of the macerating process one hundred kilos of crude jute-bast are macerated in seven hundred liters of caustic-soda lyes having a specific 60 gravity of 1.035. In the second stage one hundred kilos of crude jute-bast are macerated with the lyes expressed and discharged from the first stage with the addition of two hundred liters of fresh caustic-soda 65 lyes of the same specific gravity of 1.035 in order to increase the volume of the said lyes which remains in the one hundred kilos of jute-bast after expression. At the third stage the whole of the lyes expressed and discharged 70 from the second stage, with an addition of two hundred liters of fresh caustic-soda lyes of a specific gravity of 1.035, are used to increase the volume—i.e., to economically macerate—according to the indications furnished 75 above, three hundred kilos of crude jute-bast, which is thus treated by eleven hundred liters instead of by  $700 \times 3 = 2,100$  liters of caustic-soda lyes.

The duration of the maceration—that is to 80 say, the time during which the caustic-soda lye is allowed to act on the jute-bast in the receptacle—should amount to about from four to six hours at an ordinary temperature—that is to say, without the aid of heat. After the 85 lapse of this maceration-time of about four to six hours the macerating-lyes are drawn off from the receptacle by the discharge-cock and the macerated jute-bast is removed from the said receptacle and freed from the macerating-lyes which it may still contain by means of iron cylindrical rollers, the drawn off as well as the expressed lyes from the first stage of the operation being utilized to macerate, with the addition of fresh lyes, as indicated, the jute-bast in the second stage, 90 which is carried on in the same manner as the first stage. After the third stage of the mac-

erating process the macerating-lyes are no longer used and are thrown away.

In the chlorin process the jute-bast, macerated in the caustic-soda lyes and freed therefrom by expression, contains about seven per cent. of fixed caustic soda and is subjected to a chlorin process in a chlorin-chamber, preferably made of brickwork lined internally with enameled tiles and provided with a trellis of wooden laths or the like as a support for the macerated jute-bast, the macerated and expressed jute-bast being suspended lengthwise in the chlorin-chamber on the said trellis. As soon as this chlorin-chamber is closed gas-tight and the lead pipe, which starts from the center thereof, has been connected to the chlorin-generating apparatus chlorin-gas is admitted in the said chamber.

According to our experiments one hundred kilos of jute-bast require as much chlorin for the chlorination process as is produced by the mixture of thirty kilos of peroxid of manganese having a yield of from sixty to seventy per cent. of oxygen, sixty kilos of chlorid of sodium, and one hundred and twenty kilos of sulfuric acid at 58° Baumé. This chlorin process for the treatment of the macerated jute-bast has for its object to form a compound with the incrustations and in presence of the contents of caustic soda of the macerated and expressed jute-bast submitted according to the indications furnished under the process, as above described, to the chlorin treatment, in particular with the rosin "jutin" discovered by us in the jute-bast, which compound is subsequently entirely removed in the course of the following cold treatment owing to its being readily dissolved. After having been subjected to the chlorin process the chlorinated jute, which has now an acid reaction, is removed from the chlorin-chamber and is washed with cold water in a suitable washing-machine until the washing-water ceases to have an acid reaction, whereupon the washed jute is subjected to a process of revivification. For this purpose the chlorinated and clean-washed jute is transferred to a reservoir of sheet-iron, being placed lengthwise therein. As soon as the jute is placed in the reservoir the chlorinated jute is covered with caustic-soda lyes of a specific gravity of 1.085 until the level of the lyes is above that of the jute. One hundred kilos of chlorinated jute-bast require, according to experiments, about four hundred and seventeen liters of caustic-soda lyes of a specific gravity of 1.035 to carry out the revivification process, the lyes being left for about six hours in contact with the chlorinated jute-bast. After this time the lyes are removed from the jute-bast and as they are discharged they have assumed, in consequence of the dissolved incrustations, a dark reddish-brown color. The jute-bast left in the reservoir, which is now entirely free from incrustations and appears in the form of fine fibers, is washed in the same reservoir with cold water until the wash-

ing-water is thoroughly clean and has no alkaline reaction whatsoever. These clean-washed jute fibers are now subjected to a bleaching treatment in a bleaching - reservoir made, preferably, of cement and having its bottom covered with a wooden trellis (double bottom) or the like, so that the bleaching-lyes may come through the opening in the trellis-work uniformly in contact with every portion of the jute fibers thus laid on such trellis. As soon as the jute fibers have been transferred to the bleaching-reservoir the bleaching-lyes are poured thereon in the form of an aqueous solution of a hypochlorite of soda having a specific gravity of 0.5° Baumé until the jute fibers are covered over by the same.

By using hypochlorite of soda as bleaching means for the jute fibers we derive an advantage as compared with the bleaching means hitherto used—that is to say, with a solution of chlorid of lime—in so far that by the use of hypochlorite of soda as bleaching means no lime can adhere to the fibers—i. e., no lime particle can become fixed in the intercellular substance of the fibers—whereas in the bleaching of fibers by means of a solution of hypochlorite of lime or chlorid-of-lime lyes there was a deposit of lime on the fibers, which could not be removed by a long washing operation and which was the ultimate cause of their brittleness and rigidity. The jute fibers are left in the bleaching-bath from about four to six hours, after which the bleaching-lyes are drawn off from the jute fibers, while the latter are left in the bleaching-reservoir for another two or four hours, so as to be still further bleached. The duration of this further bleaching, as above set forth, is a matter of great importance, as the particles of bleaching-lyes still adhering to the jute fibers (hypochlorite of soda) are regenerated by the absorption of oxygen from the air and supply oxygen in a highly oxidizing state (*in statu nascente*) to the jute fibers, which oxygen or ozone acts as a powerful bleaching means, so that this subsequent bleaching permits of fully benefitting by the utilization of the bleaching process.

After the bleaching has been effected according to the indications furnished under the treatments above described the jute fibers are removed from the reservoir and are washed with cold water in a suitable washing-machine until the bleached and washed jute fibers cease to give a chlorin reaction. The bleached and well-washed jute fibers are subsequently drained and dried at a temperature of about 40° centigrade.

The crude jute fibers treated in the manner above indicated appear after being bleached and dried as a fiber, which is entirely free from incrustations or impurities, having a particularly beautiful silky gloss, and when such fibers are spun into yarns and woven into fabrics, either alone or mixed with wool and silk, they make a product hitherto unknown in the textile industries.

Having now particularly described and ascertained the nature of our said invention and in what manner the same is to be performed, we declare that what we claim is—

- 5 The herein-described process for the treatment of jute-bast and the like, consisting in first subjecting the material to mechanical means to loosen the jute and free it from tips and root ends; macerating the material thus  
10 treated without the aid of heat by subjecting it to caustic-soda lyes; next subjecting the macerated material to pressure to express the lye absorbed by the jute-bast; next subjecting the macerated material to the action of  
15 chlorin gas; washing the chlorinated jute in

cold water; subjecting the chlorinated and washed jute to the action of caustic-soda lye; again washing the jute; subjecting the purified and washed material to a bleaching process and finally washing and drying the jute 20 fibers, substantially as described.

In witness whereof we have hereunto set our hands in presence of two witnesses.

AUGUST H. PRINZ.

HERMANN HABER.

EMERICH TOMISCHKA.

JOSEF FREIHERR V. BRENNER.

Witnesses:

HENRY C. CARPENTER,  
CHAS. E. CARPENTER.